

June 3, 1924.

1,496,314

Y. IKEDA

IGNITION PELLET

Filed Feb. 19, 1923

Fig. 1.

8

Fig. 2.



Fig. 3.



Fig. 4.



Fig. 5.



INVENTOR.

BY *Yuyemon Ikeda.*

*Edward M. Kojima*  
ATTORNEY.

## UNITED STATES PATENT OFFICE.

YUYEMON IKEDA, OF GARDENA, CALIFORNIA.

## IGNITION PELLET.

Application filed February 19, 1923. Serial No. 620,064.

*To all whom it may concern:*

Be it known that I, YUYEMON IKEDA, a subject of the Emperor of Japan, residing at Gardena, in the county of Los Angeles and State of California, have invented a new and useful Ignition Pellet, of which the following is a specification.

This invention relates to ignition pellets, and has for its object the provision of an improved means for igniting combustible materials and for producing fire; the pellets being intended as a substitute for matches, and consisting of a globular pellet of combustible material, dipped in and coated with pyrophoric material, and having an outer coating of an ignitable material.

Heretofore, matches have consisted of a wooden splint, having one end coated with some ignitable composition; such matches being held by the hand of the operator during ignition and combustion of the match. To obtain a substitute which may be contained in a more limited space, or which may include a much larger number in a limited space, I have designed an ignition pellet, comprising a globular combustible material coated with pyrophoric and ignitable materials, and having a combustible capacity equivalent to the ordinary match.

In the drawings, Figure 1 is a side view embodying my invention and showing the approximate size of the igniting pellet. Fig. 2 is an enlarged and sectional view of the same. Fig. 3 is an enlarged and sectional view of a pellet having only the pyrophoric coating capable of ignition by friction with a specially prepared surface. Fig. 4 is an enlarged and sectional view of a pellet in which the combustible material and the pyrophoric material are mixed; the pellet being ignitable only with contact with a specially prepared surface. Fig. 5 is an enlarged and sectional view of a pellet having the central body portion composed of a mixture of the combustible material and pyrophoric material, and having an outer coating of readily ignitable material.

In reference to the materials herein, the combustible material includes any material or substance suitable for the main body or part of a match; the pyrophoric material designates the material commonly used for the coating of safety matches; and the ignitable material designates the material used

for making the friction tips of ordinary matches.

Referring to the drawings, the central and main portion 6, of the pellet consists of a combustible material, such as wood, felt, or compressed wicking or paper, and preferably prepared by soaking in a solution of saltpetre and lime-water, and then dried. The inner coating 7 ignites by application of fire or friction with a special surface, as used on safety matches. The outer coating 8, consists of an easily ignitable material, such as applied to the tips of ordinary matches, or of a paste made from mealed powder, phosphorus, powdered glass, and alcohol.

The main body of the pellet, being prepared in accordance herewith, will then burn for a period of time equivalent to the ordinary match; the saltpetre acting to maintain the combustion, while the lime-water determines the rate of combustion. The inner coating, ignitable by friction with only a specially prepared surface, is employed only for "safety" pellets, while the outer coating will ignite upon contact with ordinary surfaces when frictionally applied thereto. For "safety" pellets, the outer coating is omitted. Saltpetre and lime-water impart slow-burning properties. The outer coating is ignitable by a spark or friction, the inner coating by friction only.

From the foregoing description it may be seen that I have provided an improved pyrophoric pellet, adaptable for producing fire for igniting other materials, and for analogous purposes.

What is claimed is:

1. An ignition pellet, comprising an inner and globular body of a slow combustible material, an intermediate coating of a quick combustible material, and an outer envelope of frictionally ignitable material.

2. An ignition pellet comprising an inner body of a combustible material, and adapted for a slow rate of combustion, an inner ignitable and more inflammable material forming a coating on the inner body, and an outer coating of readily ignitable material thereon.

In testimony whereof, I hereunto affix my signature.

YUYEMON IKEDA.